

(No Model.)

W. F. C. M. McCARTY.  
MOLDING ARMOR PLATES.

No. 415,174.

Patented Nov. 12, 1889.



Witnesses

A. Mahon

H. M. Sterling

By his Attorney

Inventor

W. F. C. M. McCarty

*Sam J. Insabagh*

# UNITED STATES PATENT OFFICE.

WILLIAM FITZ CHARLES MASON McCARTY, OF HAGERSTOWN, MARYLAND,  
ASSIGNOR OF PART TO WILLIAM H. ASHTON AND HEMAN DUDLEY WAL-  
BRIDGE, BOTH OF WASHINGTON, DISTRICT OF COLUMBIA.

## MOLDING ARMOR-PLATES.

SPECIFICATION forming part of Letters Patent No. 415,174, dated November 12, 1889.

Application filed August 29, 1889. Serial No. 322,333. (No model.)

*To all whom it may concern:*

Be it known that I, WILLIAM FITZ CHARLES MASON McCARTY, a citizen of the United States, residing at Hagerstown, in the county 5 of Washington and State of Maryland, have invented new and useful Improvements in Molding Armor-Plates; and I do hereby declare the following to be a full, clear, and exact description of said invention, reference 10 to being had to the accompanying drawings, and to the letters of reference marked thereon, which form a part of this specification.

My invention relates to an improvement in molds for casting armor-plates for ships of 15 war, and has for its object the construction of armor-plates composed of layers of steel or other metal of different degrees of hardness, in order to more effectually resist the force of the shot projected against it.

20 My invention consists in the devices and molds for casting compound armor-plates of two or more strata of steel of different hardness by placing division-plates in the molds of fusible metal, said division-plates being 25 provided with cavities for the reception of a flux and case-hardening compound.

Referring to the drawings, Figure 1 is a top or plan view of the mold open. Fig. 2 is a view in perspective of the mold when filled. 30 Fig. 3 is also a view in perspective of the mold, showing the cavities in the division-plates. Fig. 4 is an edge view of the division-plates. Fig. 5 is a view in perspective of one of the compound plates.

35 A indicates the mold in which the plates are cast, and is composed of the sides B, bottom C, and end pieces D, the whole being held and clamped in position by rods E and end pieces F in the usual manner. The end 40 sections D of the molds are provided with grooves a to receive and sustain in a vertical position the diaphragms or plates G, and the bottom of said mold is provided with openings b, entering each compartment formed by 45 the diaphragms, which communicate with suitable fire-resisting pipes, and through which the molten metal is admitted to the different compartments of the mold.

The diaphragms or division-plates G are 50 made of a suitable metal which will melt as the molten metal is brought in contact there-

with, the sides of said plates being provided with numerous cavities c, into which is placed a fluxing and case-hardening compound, so that as the plates melt away a permanent joint is 55 formed and a plate is produced which is not only homogeneous throughout, but case-hardened and composed of two or more metals having different degrees of hardness, or a plate composed of layers of iron and steel, as may 60 be desired. The forming of the cavities in the plates causes the plates to melt away quicker at these points and allows the molten metal in each compartment to mix and have interlocking joints, which also tend to hold the 65 plates or sections forming the plates more firmly together. This process not only simplifies the manufacture of steel plates, ingots, &c., but the cost of producing them is reduced to the minimum. 70

The fluxing or cementing compound is filled into the cavities in the plates G, and is composed of the following ingredients: yellow prussiate of potash, one-fourth; cyanide of potash, one-fourth; animal charcoal, one-half. 75 These ingredients are mixed into a paste with either glycerine, glucose, or any other suitable vehicle to form a paste, which is filled into the cavities of the plates and well dried to harden the flux in position. 80

The molten masses of metal of which the plates are formed are subjected to a vacuum to remove all the occluded gases, so that a homogeneous mass may be formed free from blow-holes, gases, &c., thus producing a 85 molecular structure more dense, and consequently stronger, than by any other process, this process of vacuum treatment being embraced in my patent, No. 404,723, of June 4, 1889.

What I claim, and desire to secure by Letters Patent, is—

A mold for casting armor-plates, divided into sections by fusible plates provided with cavities containing a flux and case-hardening compound. 95

In testimony whereof I affix my signature in the presence of two subscribing witnesses.

WILLIAM FITZ CHARLES MASON McCARTY.

Witnesses:

GEORGE CAMPION,  
WM. LOGAN.